

## UNITED STATES PATENT OFFICE

2,092,007

## TREATMENT OR MANUFACTURE OF CELLULOSE ESTER MATERIAL

Robert Wighton Moncrieff and Frank Brentnall Hill, Spondon, near Derby, England, assignors to Celanese Corporation of America, a corporation of Delaware

No Drawing. Application December 6, 1934, Serial No. 756,283. In Great Britain December 12, 1933

15 Claims. (Cl. 8—20)

This invention relates to the manufacture or treatment of filaments, threads, yarns, ribbons and the like having a basis of cellulose acetate or other organic ester of cellulose.

5 It is known to saponify cellulose ester materials and also to stretch such materials with a view to increasing their tenacity. We have now found a means of stretching the materials to a considerable extent and of saponifying them simultaneously. When it is attempted to stretch in an ordinary alkaline saponifying bath, for instance a caustic soda bath, serious difficulties are encountered. Apart from the difficulty of effecting a substantial degree of stretch in such baths, even 10 in the presence of a softening agent for the material, there is the difficulty that such stretch as is effected tends to render the materials brittle and/or harsh to the touch and in other respects to injure their serimetric properties. We have 15 found that by treating cellulose acetate threads and like materials in a bath containing a non-metallic base, for example mono-methylamine, which bath is capable of softening the base of the materials, stretching may actually be effected simultaneously with saponification with most valuable results. The process of the invention makes 20 it possible to obtain from ordinary cellulose acetate materials in a single operation, materials of high tensile strength, good extensibility and low 25 denier. These materials may have an affinity for cotton dyes as well as for cellulose ester dyes. The process can be carried out rapidly and continuously. The saponification effected may extend to a considerable depth beneath the surface, 30 or even throughout the whole section of the materials, and acetone-solubility may be decreased considerably with relatively little loss in weight. The process also enables other desirable properties 35 of saponified cellulose esters on the one hand, and of stretched materials on the other, to be obtained. Thus, the safe ironing point of the materials is considerably higher than that of ordinary cellulose ester materials, and they exhibit an enhanced 40 resistance to the delustring action of hot aqueous liquids.

The invention is of particular importance in connection with the treatment of filaments, threads, ribbons, fabrics and like materials having a basis of cellulose acetate and will be described with special reference to the treatment of such materials.

45 The materials treated may be made by any suitable dry or wet spinning method. Where high 50 tenacity is required in the final products it is of particular advantage to produce the filaments and

the like by wet spinning methods in the course of which they are stretched to a considerable extent, or to soften and stretch the materials after their production whether by a wet or a dry spinning process. By applying the process of the invention to materials which have been stretched considerably, for example to 200% of their original length or even more, materials of particularly valuable serimetric properties are obtainable.

5 The non-metallic base preferably comprises mono-methylamine. Other strong aliphatic organic bases, for example ethylamine, propylamine, amylamine and triethylamine, may also be employed. Again, somewhat weaker bases of the same series, for example trimethylamine and allylamine, may be used. Further, considerably stronger bases of the same series may be employed, even very strong bases such as tetramethyl ammonium hydroxide, provided care be taken to avoid damaging the materials. Again, amines 10 containing more than one amino group, and particularly aliphatic diamines of relatively low molecular weight, for example ethylene diamine, symmetrical dimethyl ethylene diamine, mono-methyl ethylene diamine, and propylene diamine 15 may also be used. Preferably at least one of the amino groups of such amines should be unsubstituted or mono-substituted. Amines containing more than two amino groups may also be employed, for example 1,2,3-triamino propane. The 20 effect of one or more hydroxy groups in the amine appears to be to favour the penetration of the materials by the saponifying agent, and with this object in view substances of the type of  $\alpha\gamma$ -diamino- $\beta$ -hydroxy propane may be used with advantage. Again, bases of the heterocyclic series, 25 for example piperidine may be used. The bath may contain substances adapted to accelerate the action of the non-metallic base. Various inorganic substances which may be employed for this 30 purpose are mentioned in U. S. application S. Nos. 756,282, 756,284, and 756,285, filed December 6, 1934. Among such substances special mention 35 may be made of caustic soda and of copper in solution in connection with saponification by means of 40 methylamine or other lower aliphatic amines.

The swelling agent is preferably a swelling 45 agent of relatively high solvent power for the base of the materials. Thus in the case of cellulose acetate, we may employ for example, acetone, diacetone alcohol, cyclohexanol, cyclohexanone, methyl cyclohexanone, dioxane or 50 methylene ethylene ether.

The process is preferably effected by drawing 55 the materials through an aqueous bath contain-

ing the swelling agent and non-metallic base and stretching them while they are passing through the bath. It is of advantage to treat a large number of ends at one time, drawing them through the bath in warp formation, that is in substantially parallel relationship one with another and in the same plane, by means of a series of rollers, reeds being employed where necessary to maintain the warp formation. The speeds of successive sets of rollers may increase progressively along the path of the materials so as to insert progressively increasing stretch. On the other hand, stretching may be effected in stages between which the materials are allowed to relax under substantially no tension. Thus, for example, the materials may pass from the feed rollers through a set of rollers rotating at a higher speed so as to impart a stretch, then through a set rotating at a slightly lower speed than the second set, and from thence through a set rotating at a higher speed than the second set. The materials are preferably stretched to 150 or 200% or more of their original length.

The concentration of swelling agent and base in the bath and the temperature of the bath may vary according to the extent of saponification and of stretch to be effected. Generally speaking, temperatures of the order of 15-20° C. or 25-35° C. will be found convenient. For the swelling agent an aqueous concentration between 20 and 40 or 60% will generally be found suitable. In the case of the non-metallic base suitable concentrations will generally be found between 2 and 5 or 10%.

35 The degree of saponification effected may be sufficient to produce a loss in the acetyl content of the ester of 10-15% or even less, but is preferably somewhat greater, for example sufficient to produce a loss in the acetyl content of 20-25%.

40 The following example illustrates the invention:—

*Example*

Cellulose acetate yarn is drawn in warp formation through an aqueous bath containing 35-45% dioxane. The speed of travel of the material is such that it is in contact with the bath for 1-3 minutes and is stretched to 150-200% of its original length during the passage through the bath. The bath contains mono-methylamine in a proportion depending upon the amount of saponification to be effected. On leaving the bath the materials pass through a short washing bath and then over heated drums to suitable winding means.

55 Although the invention has been described with particular reference to the treatment of materials having a basis of cellulose acetate, it is also applicable to the treatment of other materials containing saponifiable esters of cellulose, for example cellulose formate, propionate, butyrate, ethyl cellulose acetate, oxyethyl cellulose acetate and nitrocellulose acetate.

What we claim and desire to secure by Letters Patent is:—

65 1. Process for the manufacture of improved artificial materials, which comprises softening and partially saponifying filaments, threads, ribbons and like materials having a basis of organic esters of cellulose by treatment with a swelling bath which contains a non-aromatic nitrogenous organic base which contains less than seven carbon atoms, and stretching the softened materials during saponification.

70 2. Process for the manufacture of improved artificial materials, which comprises softening

and partially saponifying filaments, threads, ribbons and like materials having a basis of organic esters of cellulose by treatment with a swelling bath which contains a nitrogenous organic base, having less than seven carbon atoms, of dissociation constant at least as high as trimethylamine, and stretching the softened materials during saponification. 5

3. Process for the manufacture of improved artificial materials, which comprises softening and partially saponifying filaments, threads, ribbons and like materials having a basis of cellulose acetate by treatment with a swelling bath which contains a non-aromatic nitrogenous organic base which contains less than seven carbon atoms, 15 and stretching the softened materials during saponification. 15

4. Process for the manufacture of improved artificial materials, which comprises softening and partially saponifying filaments, threads, ribbons and like materials having a basis of cellulose acetate by treatment with a swelling bath which contains a water-soluble nitrogenous base containing less than seven carbon atoms in which each carbon atom that is directly attached to a 25 nitrogen atom is directly attached to three other atoms apart from said nitrogen atom, and stretching the softened materials during saponification. 20

5. Process for the manufacture of improved artificial materials, which comprises simultaneously softening and partially saponifying filaments, threads, ribbons and like materials having a basis of organic esters of cellulose by drawing the materials through an aqueous softening bath containing a neutral swelling agent for the 35 organic ester of cellulose and a non-aromatic nitrogenous organic base which contains less than seven carbons atoms, and stretching the softened materials during their passage through said bath. 30

6. Process for the manufacture of improved artificial materials, which comprises simultaneously softening and partially saponifying filaments, threads, ribbons and like materials having a basis of organic esters of cellulose by drawing the materials through an aqueous softening bath 45 containing a neutral swelling agent for the organic ester of cellulose and mono-methylamine, and stretching the softened materials during their passage through said bath. 40

7. Process for the manufacture of improved artificial materials, which comprises simultaneously softening and partially saponifying filaments, threads, ribbons and like materials having a basis of cellulose acetate by drawing the materials through an aqueous softening bath containing a 55 neutral swelling agent for cellulose acetate and a lower aliphatic amine, and stretching the softened materials during their passage through said bath. 50

8. Process for the manufacture of improved artificial materials which comprises simultaneously softening and partially saponifying filaments, threads, ribbons and like materials having a basis of cellulose acetate by drawing the materials through an aqueous softening bath containing a 60 neutral swelling agent for the cellulose acetate and mono-methylamine, and stretching the softened materials during their passage through said bath. 65

9. Process for the manufacture of improved artificial materials which comprises simultaneously softening and partially saponifying filaments, threads, ribbons and like materials having a basis of cellulose acetate by drawing the materials through an aqueous softening bath 70 containing a neutral swelling agent for the cellulose acetate and mono-methylamine, and stretching the softened materials during their passage through said bath. 75

taining a neutral swelling agent for the cellulose acetate and ethylene diamine, and stretching the softened materials during their passage through said bath.

5 10. Process for the manufacture of improved artificial materials, which comprises softening and partially saponifying filaments, threads, ribbons and like materials having a basis of organic esters of cellulose by treatment with a swelling bath

10 which contains a non-aromatic nitrogenous organic base which contains less than seven carbon atoms, so as to effect a loss of 10-25% of the acidyl content, and stretching the softened materials during saponification.

15 11. Process for the manufacture of improved artificial materials, which comprises softening and partially saponifying filaments, threads, ribbons and like materials having a basis of organic esters of cellulose by subjecting the materials to the

20 action of a swelling bath containing a water-soluble nitrogenous base containing less than seven carbon atoms in which each carbon atom that is directly attached to a nitrogen atom is directly attached to three other atoms apart from

25 said nitrogen atom and a small quantity of a mineral alkali, and stretching the softened materials during saponification.

12. Process for the manufacture of improved artificial materials, which comprises softening and

30 30 partially saponifying filaments, threads, ribbons and like materials having a basis of organic esters of cellulose by subjecting the materials to the action of a swelling bath containing a non-aromatic nitrogenous organic base which contains

35 less than seven carbon atoms and a small quan-

5 tity of copper in solution, and stretching the softened materials during saponification.

13. Process for the manufacture of improved artificial materials, which comprises simultaneously softening and partially saponifying filaments, threads, ribbons and like materials having a basis of cellulose acetate by drawing the materials through an aqueous softening bath containing a neutral swelling agent for cellulose acetate, mono-methylamine and a small quantity of copper in solution, and stretching the softened materials during their passage through said bath.

10 14. Process for the manufacture of improved artificial materials, which comprises drawing filaments, threads, ribbons or like materials having 15 a basis of cellulose acetate, in warp formation through an aqueous dioxane bath, containing mono-methylamine, so as to effect a relatively deep-seated saponification resulting in a loss of 10-20% of the acetyl content, and stretching the 20 materials to at least 150% of their original length during their passage through said bath.

15. Process for the manufacture of improved artificial materials, which comprises drawing filaments, threads, ribbons or like materials having 25 a basis of cellulose acetate, in warp formation through an aqueous acetone bath containing mono-methylamine, so as to effect a relatively deep-seated saponification resulting in a loss of 10-20% of the acetyl content and stretching the 30 materials to at least 150% of their original length during their passage through said bath.

ROBERT WIGHTON MONCRIEFF.

FRANK BRENTNALL HILL.

35